

Jan. 26, 1926.

1,570,617

L. G. COPEMAN

METHOD OF REFRIGERATOR MANUFACTURE

Filed April 6, 1925

3 Sheets-Sheet 1



Jan. 26, 1926.

1,570,617

L. G. COPEMAN

METHOD OF REFRIGERATOR MANUFACTURE

Filed April 6, 1925

3 Sheets-Sheet 2



INVENTOR.

Lloyd G. Copeman

BY

Stuart L. Barnes

ATTORNEY.

Jan. 26, 1926.

1,570,617

L. G. COPEMAN

METHOD OF REFRIGERATOR MANUFACTURE

Filed April 6, 1925

3 Sheets-Sheet 3



Fig. 4

INVENTOR.

Lloyd G. Copeman

BY

Stuart C. Barnes

ATTORNEY.

Patented Jan. 26, 1926.

1,570,617

# UNITED STATES PATENT OFFICE.

LLOYD G. COPEMAN, OF FLINT, MICHIGAN.

## METHOD OF REFRIGERATOR MANUFACTURE.

Application filed April 6, 1925. Serial No. 21,002.

To all whom it may concern:

Be it known that I, LLOYD G. COPEMAN, a citizen of the United States, residing at Flint, in the county of Genesee and State of Michigan, have invented certain new and useful Improvements in Methods of Refrigerator Manufacture, of which the following is a specification.

This invention relates to a method of refrigerator manufacture and has for its object means for moulding a complete composite refrigerator shell with one set of mould sections. Obviously other articles as well could be manufactured by the same method.

In constructing any refrigerator with a composite shell, whether the shell is composed of two kinds of mouldable material or a material moulded over a wood core, it necessitates considerable work. In coating a refrigerator core with artificial stone or a finishing coat, it is necessary to use two complete sets of moulds as the refrigerator core must be first moulded and then placed into another set of moulds so that the layer of artificial stone which covers the core may be moulded or cast thereon.

In the drawings:

Fig. 1 is a view showing the mould in section, and the means for separating the mould section so that the same may be sprayed with a relatively thin outer layer of stone or other finishing material.

Fig. 2 is a vertical sectional view showing the mould sections drawn together in readiness for pouring the refrigerator core.

Fig. 3 is a similar view showing the refrigerator core poured into the moulds.

Fig. 4 is a perspective view of the completed refrigerator with parts broken away to show the composite character of the shell.

*a* designates the side walls of the outer mould, which are secured to the bottom mould section *b*, provided with the openings *c* in which the inner mould sections or cores *d* are fitted when the same are drawn or fitted together. These inner mould sections or cores are supported on the plunger *e* which works in the cylinder *f*; compressed air or hydraulic pressure may be exerted on the end of the plunger for raising the same to any height desired, it being necessary that these cores be raised to such a height that the operator can spray the inside of the outer mould section with a spray gun *g*. It would be impossible to spray the matrices of the mould sections were it not for the fact that the

same can be sprayed and then drawn together and correctly positioned with respect to each other, without necessitating an adjustment every time the mould sections are separated.

The first step in the method is the coating of the matrices of the mould sections with an oxy-chloride cement composition. This coating forms an outer layer *h* of cement which when hardened forms a very good artificial stone. This composition is preferably composed of a mixture of magnesium oxide 25%, (silica) 50% and sand 25%, all percentages calculated by weight. To this dry mix is added sufficient magnesium chloride in solution of 26 Bé. gravity, to make the mixture suitable for spraying in a spray gun. I preferably spray this material on the mould sections as it is the most convenient and practical way in which to coat the same, but obviously this material could be coated on the matrices of the mould sections in other ways if desirable. Obviously a finishing coating containing other materials could be used depending on the article and the use to which it is put.

The next step in the operation is the dropping of the inner mould sections or cores into position within the outer mould. Such a position is shown in Fig. 2 which shows the inner cores spaced from the walls of the outer mould section, the surface of the mould sections carrying this relatively thin layer of artificial stone or finishing coat which may or may not have completely hardened. This layer could be hardened completely before the mould sections are fitted together, or it is probable that after the artificial stone composition is sprayed on the moulds the same will be immediately fitted together. The next step is the pouring of a plastic filler in the space between the moulds, which will completely fill the space, as shown in Fig. 3, between the layers of finishing material, which are coated on the matrices of the mould sections.

This plastic filler which is poured in the moulds preferably forms a core for the refrigerator shell which is relatively light in weight, due to the composition of the same, and possesses a high resistance to the conductivity of heat. This plastic filler is preferably composed of 60% magnesium oxide, by weight, 30% cork dust, by weight, and 10% glue dissolved in water. This mixture is mixed with sufficient water

to make the same a good pouring mixture. After being poured in the mould and allowed to set, it becomes very hard and strong, yet quite light, due to the large percentage of cork contained therein. This insulating core may be poured in the mould before the outer oxy-chloride cement has hardened, and both the plastic filler and the outer finishing coat allowed to harden 10 at the same time, or the finishing coat may be first allowed to set and harden before pouring the refrigerator core or filler.

In spraying the outer layer on the outer mould section, the inside surface of the 15 layer is preferably left rather rough. In other words, it has an irregular contour, so that when the inner core is poured in it fills all the valleys in the irregular surface of the outer finishing layer, thereby serving to 20 key the inner core and outer layer together.

What I claim is:

1. A method of making a refrigerator or other article of manufacture, which comprises the coating of the moulding surfaces 25 of the outer and inner mould sections with a relatively thin layer of finishing material, and the pouring of a plastic filler in said mould to form a composite shell structure.

2. A method of making a refrigerator or 30 other article of manufacture, which comprises the coating of the moulding surfaces of an outer and inner mould section with a relatively thin layer of oxy-chloride cement, and the pouring of a plastic filler of heat- 35 insulating material in said mould between the layers of oxy-chloride cement to form a composite heat-insulating refrigerator shell.

3. The method of making a refrigerator or other article of manufacture, which comprises the spraying of the moulding surfaces 40 of outer and inner mould sections with a relatively thin layer of finishing material, and the pouring of a plastic filler of heat-insulating material in said mould between the

layers of finishing material sprayed on the 45 mould sections to form a composite refrigerator shell when dried and hardened.

4. A method of making a refrigerator or other article of manufacture, which comprises the coating of the moulding surfaces 50 of an inner and outer mould section with a relatively thin coating of finishing material while said mould sections are separated, the moving of one mould section with respect to the other to bring the same together one 55 within the other, and the pouring of a plastic filler in said mould between the finishing coatings on the matrices of the mould sections to form a composite shell structure.

5. A method of making a refrigerator or 60 other article of manufacture, which comprises the coating of the moulding surfaces of an inner and outer mould section with a relatively thin coating of finishing material the surface of which has an irregular contour, and the pouring of a plastic filler in 65 said mould to form a composite shell structure, the plastic filler filling the crevices in the irregular surface of the outer finishing coating and serving to key the filler and 70 outer finishing coating together.

6. A method of making a refrigerator or other article of manufacture, which comprises the coating of the moulding surfaces of an inner and outer mould section with a relatively thin layer of artificial stone the 75 coating of a plurality of inner mould sections or cores with a relatively thin layer of artificial stone, the telescoping of said inner cores within the outer mould and fitting the same together, and the moulding of a plastic filler of heat-insulating material in 80 said mould and between the layers of stone coats to form a composite refrigerator shell when allowed to set and harden.

In testimony whereof I have affixed my signature.

LLOYD G. COPEMAN.